

# UNITED STATES PATENT OFFICE.

MADELEINE KUESS, OF TUNIS, TUNIS.

## SOAP AND PROCESS OF MAKING THE SAME.

No. 830,332

Specification of Letters Patent.

Patented Sept. 4, 1906.

Application filed January 12, 1904. Serial No. 188,770.

*To all whom it may concern:*

Be it known that I, MADELEINE KUESS, of No. 2 Rue Gharnouta, Tunis, Tunis, have invented certain new and useful Improvements in the Manufacture of Soap; and I do hereby declare the following to be a full, clear, and exact description of the invention, such as will enable others skilled in the art to which it appertains to make and use the same.

This invention relates to the manufacture of soap; and its special object is to produce a soap from petroleum or mineral oils.

Hitherto the chemical union of petroleum and other mineral oils with other ingredients to produce soap has been considered impossible, and, moreover, the disagreeable odor usually present in mineral oils has prevented their employment in the soap and perfume industries. It is true that heretofore certain semiliquid emulsions containing petroleum have been tried for the purpose of cleaning long-haired skins; but the inflammability and the disagreeable smell of these emulsions have been a serious obstacle to their general adoption in the arts.

It is not the aim of the present invention to prepare an emulsion of mineral oil or a mere mechanical mixture of the same with soap made from fats or resins; but this invention has for its object the production of a true soap from mineral oil or petroleum and, moreover, the production of a compound of petroleum or mineral oil and alkali which is free from the objectionable odors and dangerous inflammable properties inherent in the aforesaid emulsions.

With these objects in view my invention involves the addition of hydrochloric acid to a mixture of fat or of resin and fat and mineral oil in which the fat or fat and resin have been saponified by alkali. My invention, moreover, involves the addition of a further quantity of alkali to the soap mass after the treatment of all or a part of the mineral oil by the hydrochloric acid, said further addition of alkali serving to alter the hydrocarbons of the mineral oil. Under these conditions a soap may be produced from the petroleum or mineral oil and which after the lapse of a short period of time will have completely lost the odor of petroleum.

My invention, moreover, consists in the product resulting from the indicated process—namely, a soap containing chemically-bound mineral oil in contradistinction to the

old forms of soap, which contained free, uncombined mineral oil; and my invention consists in such other features and methods as will be hereinafter set forth and pointed out in the claims.

Of course it is understood that the term "fats" as herein employed is broad enough to include solid and liquid fats or oils.

Soap obtained from mineral oil under this invention dissolves in water like soaps obtained from fats or fatty oils. On being melted by heat it liquefies like ordinary soaps and becomes formed into soap again on being cooled without showing any trace of decomposition. When first made, the soap obtained from mineral oil still retains a smell; but after a few days all smell of petroleum disappears, gradually giving place to a faint, pleasant perfume. Moreover, this mineral-oil soap can be perfumed as required like other soaps.

The quantitative proportions of materials necessary for the purpose of accomplishing the desired result depend on the quality of the mineral oils and in consequence vary for every oil. To transform a small quantity of mineral oil, these proportions must be increased, and they become definite proportions only when the quantity of mineral oil to be treated is a hundred liters or more. To simplify the description of the process, let ten liters of American or Atlantic petroleum (also known as "kerosene") weighing eight hundred grams to the liter be taken as the standard.

I take ten liters of petroleum, which for the purposes of this calculation may be assumed to weigh just one kilogram per liter—that is, ten kilograms in all. I pulverize one kilogram five hundred grams of resin or any of its equivalents—such as tar, rosin, or any hydrocarbon of the class  $C_nH_{2n-4}$  (comprising the terpenes)—that is to say, fifteen per cent., supposing that a liter weighs one kilogram. The resin is then added to the petroleum, stirring continuously till the resin is dissolved, which takes place after an hour or two. All heating is to be avoided. Having incorporated the resin, one kilogram five hundred of beef fat or any other animal fat are melted over a slow fire. When the fat is quite liquid, it is taken from the fire and poured into the mass, (petroleum and resin,) stirring well. The mixture is then left for two hours, being stirred from time to time only. Six hundred and thirty grams of

caustic soda ( $\text{NaHO}$ ) are dissolved with the aid of heat in one liter three hundred centiliters of water—that is to say, the soda is taken in the ratio of five per cent. of the substance employed (always supposing in the calculations that a liter of petroleum weighs one kilogram) and is dissolved in water in the ratio of ten per cent. of all of the materials making up the entire mass. The hot liquid or lye thus obtained is then poured into the mass comprising the petroleum resin and fat, and the same is stirred constantly until the mass has become semi-solid—that is to say, has formed a thickened pulp. When the mass is semisolid, there are added gradually and preferably, drop by drop, so to speak, three hundred and twenty-five centiliters of hydrochloric acid while stirring the mass vigorously. This amount of hydrochloric acid corresponds to two and a half per cent. of the whole amount. The mass by this action and addition becomes intensely heated and is again liquefied, and it will be seen that thereby the petroleum becomes thoroughly combined with the alkali and incorporated with the saponified resin and fat. It is best to stir the mass and then to leave it until it becomes quite cool. It will be seen from the above that the amount of alkali added is more than necessary to bind or saponify the fat and resin, the remainder which is left over after such saponification serving to chemically bind a part or all (in the present instance all) of the mineral oil or petroleum. Thereupon further alkali is added by taking three hundred and twenty-five grams of caustic soda ( $\text{NaHO}$ ) and dissolving it with the aid of heat in one liter three hundred centiliters of water—that is to say, two and a half per cent. of soda in ten per cent. of water. Pour the hot liquid into the mass while stirring. Then leave the mass for four or five hours, stirring the same from time to time. The mass thereby becomes compact, forming into large lumps, and is ready to be boiled.

It is better to leave the soap for one or two days to give it time to form completely, whereupon it is dissolved over a slow fire. This soon causes it to become liquid, whereupon it is taken away and allowed to cool. It is then put into a copper and boiled for four hours. Then it is poured into the molds, allowed to cool, and dry in the shade exactly as with other soaps. The resultant soap will be found to be slightly yellow. It has great cleansing properties and is a powerful antiseptic.

If it is desired to obtain a white soap, instead of putting it in a copper it must be boiled with a large quantity of water and be continuously stirred, after which it is allowed to cool. The soap will then be found to float, the yellow coloring-matter remaining in the water. The soap thus prepared is quite white, but contains a good deal of

water. Instead of dissolving it in a salt bath, as is done with ordinary soaps, it is better to remove the water by compression. The soap is then melted over a slow fire and run into the molds. The soap made from petroleum can readily be mixed with a little palm-oil or palm-oil soap, extract of quillai or of saponin in order to make the soap lather. Palm-oil is the best, as it hardens the soap as well as makes it lather. 75

If a hundred liters of petroleum be used, only ten per cent. of resin or tar, ten per cent. of fat, five per cent. of soda, ( $\text{NaHO}$ ), and one per cent. of hydrochloric acid are employed.

Petroleum soap can also be made without the resin, only adding fat; but if the soap forms badly the quantity of caustic soda must be doubled and a disproportionate quantity of fat put in. The same conditions 85 would arise if resin alone were employed.

Having fully described my invention, what I claim as new, and desire to secure by Letters Patent of the United States, is—

1. In the manufacture of soap, the process 90 which consists in adding hydrochloric acid to a mixture comprising mineral oil and saponified fat.

2. In the manufacture of soap, the process 95 which consists in adding hydrochloric acid to a mixture comprising mineral oil and saponified fat and resin.

3. In the manufacture of soap, the process 100 which consists in adding caustic alkali to a mixture comprising mineral oil and fat, and then adding hydrochloric acid to the whole.

4. In the manufacture of soap, the process 105 which consists in adding caustic alkali to a mixture comprising mineral oil, fat and resin, and then adding hydrochloric acid to the whole.

5. In the manufacture of soap, the process 110 which consists in adding hydrochloric acid to a mixture comprising mineral oil and saponified fat, and then adding alkali to the resultant mass.

6. In the manufacture of soap, the process 115 which consists in adding hydrochloric acid to a mixture comprising mineral oil and saponified fat and resin, and then adding alkali to the resultant mass.

7. In the manufacture of soap, the process 120 which consists in adding caustic alkali to a mixture comprising mineral oil and fat, then adding hydrochloric acid to the whole, and then adding more caustic alkali to the resultant product.

8. In the manufacture of soap, the process 125 which consists in adding caustic alkali to a mixture comprising mineral oil, fat and resin, then adding hydrochloric acid to the whole, and then adding more caustic alkali to the resultant product.

9. In the manufacture of soap, the process 130 which consists in dissolving resin in mineral

oil and adding thereto melted or liquid fat, then adding a bath of more than sufficient caustic alkali to saponify the resin and fat and allowing to stand and then gradually adding hydrochloric acid to the whole.

5 10. In the manufacture of soap, the process which consists in dissolving resin in mineral oil and adding thereto melted or liquid fat, then adding a bath of more than sufficient caustic alkali to saponify the resin and fat and allowing to stand, then gradually adding hydrochloric acid to the whole, and finally adding another quantity of an alkaline bath to the resultant mass after cooling.

15 11. In the manufacture of soap, the process which consists in dissolving resin in mineral oil and adding thereto hot melted or liquid fat and allowing such mixture to stand, then adding a hot bath of more than sufficient caustic alkali to saponify the resin and the fat, stirring and allowing to stand, then, when the mass has become partially solid, adding gradually hydrochloric acid and stirring.

20 25 12. In the manufacture of soap, the process which consists in dissolving resin in mineral oil and adding thereto hot melted or liquid fat and allowing such mixture to stand, then adding a hot bath of more than sufficient caustic alkali to saponify the resin and the fat, stirring and allowing to stand, then

when the mass has become partially solid adding gradually hydrochloric acid and stirring and finally adding another quantity of a hot alkaline bath to the resultant mass after cooling, allowing to stand for a sustained period of time and then boiling the whole.

35 13. In the manufacture of soap, the process which consists in saponifying fat and resin in the presence of a hydrocarbon, adding an acid and resaponifying with alkali.

14. A soap containing chemically altered and combined hydrocarbon homogeneously distributed throughout its mass, said soap remaining homogeneous when heated and when 40 boiled with water.

15. A soap comprising saponified fat and resin and a chemically altered and combined hydrocarbon, all in a state of homogeneous admixture, said soap remaining homogeneous when heated and when boiled with water.

45 16. A soap containing mineral oil and also containing saponified fat and resin recovered from a previous saponification in presence of such mineral oil.

50 In witness whereof I have hereunto set my hand in presence of two witnesses.

MADELEINE KUESS, (NÉE SOLLEY.)

Witnesses:

L. PARODI,  
N. ROTTER.